

## UNITED STATES PATENT OFFICE

WILLARD DE C. CRATER, OF SUCCASUNNA, NEW JERSEY, ASSIGNOR TO HERCULES POWDER COMPANY, OF WILMINGTON, DELAWARE, A CORPORATION OF DELAWARE

## CHARGE FOR BLASTING CAPS

No Drawing.

Application filed August 13, 1929. Serial No. 385,696.

My invention relates to an improvement in blasting, charges for caps such as are customarily used in connection with commercial explosives.

As is well known, blasting caps are used to effect the detonation or firing of commercial explosives, such as dynamites, permissible explosives, etc., which require for their detonation or firing a primer charge as compared 10 with mere ignition, as in the case of firing, for example, black powder. Heretofore various substances and mixtures of substances have been utilized in the charging of blasting caps, however, the prior caps have not been entirely 15 satisfactory from all standpoints.

Now, in accordance with my invention, I have discovered that a superior blasting cap is provided where the cap is charged with nitrolactose. In accordance with my invention 20 the nitrolactose is desirably associated with some substance capable of acting as an initial primer, the initial primer being superimposed on the nitrolactose or being admixed therewith.

25 In producing a blasting cap in accordance with my invention the nitrolactose may be used in association with any desired substance or compound which will be effective as an initial primer, such as, for example, fulminate-chlorate, diazo dinitrophenol, lead 30 azide, etc. and, as has been indicated, the substance or compound used as an initial primer may be superimposed on the nitrolactose, or may be admixed therewith.

35 In the production of a cap in accordance with my invention, for example, the cap shell may be first charged with say about 0.5 g. of nitrolactose and there may then be superimposed thereon say about 0.4 g. of 40 fulminate-chlorate, the charge being suitably compressed in the shell.

If desired, in charging a cap with nitrolactose as, for example, fulminate-chlorate, the nitrolactose and fulminate-chlorate may 45 be intermixed, preferably intimately, and the mixture charged into the cap shell and suitably compressed.

It will be understood that the nitrolactose may be used in connection with any suitable 50 substance which will act as an initial primer

other than fulminate-chlorate, as, for example, lead azide, diazo dinitrophenol, etc. the initial primer substance being, for example, superimposed on the nitrolactose or admixed therewith.

It will be noted that the cap in accordance with my invention will possess characteristics equal to or superior to caps heretofore known, and particularly as regards grams of sand crushed in the sand test and in their capacity 55 for efficiently detonating commercial explosives, as for example, dynamites, etc.

It will be understood that my invention from the broad standpoint involves the use 60 of nitrolactose as an ingredient of a charge for blasting caps, the nitrolactose being desirably associated in a practical manner with a substance adapted to act as an initial primer. It will also be understood that the nitrolactose may be used in association, as in 65 admixture with another explosive not necessarily a primer, as for example, tetryl.

What I claim and desire to protect by Letters Patent is:

1. In a blasting cap a charge including 75 nitrolactose as an ingredient.

2. In a blasting cap a charge including nitrolactose and a substance capable of acting as a primer for the nitrolactose.

3. In a blasting cap a charge including 80 nitrolactose and a substance capable of acting as a primer for the nitrolactose superimposed on the nitrolactose.

4. In a blasting cap a charge including 85 nitrolactose and fulminate-chlorate.

5. In a blasting cap a charge including nitrolactose and fulminate-chlorate superimposed on the nitrolactose.

In testimony of which invention, I have 90 hereunto set my hand, at Kenvil, N. J., on this 7th day of August, 1929.

WILLARD DE C. CRATER.

55

60

65

70

80

85

95

100